

Patented Oct. 23, 1928.

1,688,695

# UNITED STATES PATENT OFFICE.

GUSTAVUS J. ESSELEN, JR., OF SWAMPSCOTT, AND MARK W. WEISS, OF BOSTON, MASSACHUSETTS, ASSIGNORS TO THE DELAWARE, LACKAWANNA & WESTERN COAL CO., OF NEW YORK, N. Y., A CORPORATION OF NEW JERSEY.

## COAL.

No Drawing. Application filed December 28, 1927. Serial No. 243,203.

This invention relates to carbonaceous fuel of distinctive appearance which distinguishes it from ordinary fuel of the same class. The invention is applicable to anthracite and 5 bituminous coal in various sizes and to briquettes, coke and the like.

Carbonaceous fuel of the character described comes to the market in varying qualities and grades. The quality of such fuels 10 cannot be determined by appearance and consequently the consumer is often supplied with inferior grades at the prices of superior grades. Unscrupulous dealers sometimes 15 take advantage of consumers by delivering low grade fuel as the product of some well known producer having a reputation for the high quality of his product and both the consumer and the producer are thus defrauded.

20 It is the object of the present invention to avoid the possibility of substitution by imparting to the fuel a distinctive color and to provide a method whereby the appearance of the fuel can be modified at reasonably low 25 cost.

Other objects and advantages of the invention will be apparent by reference to the following specification in which the preferred embodiments are described.

30 To fulfill the requirements and to meet the purpose of the invention the fuel is superficially coated with a suitable coloring material. The coating need not be uniform nor is it necessary to apply it to all of the 35 exposed surface of the fuel. Coal and similar fuels are handled in bulk and it has been found that a relatively light application of the color medium will give the bulk fuel a distinctive appearance. The purpose may be 40 accomplished even by applying the color to only a portion of the fuel and by mixing colored with uncolored fuels in suitable proportions.

45 For the purpose of the invention various coloring materials may be employed and such materials may be applied in different ways. The coloring materials and the method of application should be such that the fuel will retain its distinctive appearance during 50 repeated handling and exposure to water incident to transportation. Numerous coloring materials suitable for the purpose are available.

Among the available materials are water-

insoluble pigments or colors with or without 55 binders, water-soluble coloring material with or without binders, and oil-soluble coloring material with or without binders. Colors which are soluble in other media such as alcohol, acetone, benzol, toluol, etc., and certain 60 dyes which are adapted to be fixed with mordants, may be used. Such materials may be applied to the fuel in various ways, for example, by conveying the fuel through a liquid suspension or solution of the coloring 65 material or by spraying the suspension or solution of coloring material upon the fuel in the conveyor. Another method of application is to place the fuel in a suitable receptacle containing the suspension or solution or to spray 70 the suspension or solution over a pile of the fuel in such a receptacle. In each case provision should be made to drain the excess liquid from the fuel so that waste is avoided. The fuel may then be dried, but this is not necessary. Such operations may be conducted as 75 a part of the usual washing procedure. It is also possible to dust certain colors or pigments with or without binders on the fuel while the latter is in a moistened condition, 80 the color being fixed when the fuel is dry.

No attempt is made herein to describe every possible adaptation of the invention. The examples hereinafter mentioned are, therefore, illustrative of the invention and 85 it is to be understood that various changes and modifications can be made in the nature of the coloring material employed and in the method of application thereof within the scope of the invention. 90

As a typical example of a satisfactory procedure the pigment commercially known as ultra-marine or "Celestial Blue", consisting of a complex compound of sodium, aluminum, silicon, sulphur and oxygen, may be 95 used with desirable results. The pigment, preferably in finely divided condition, is suspended in water. The proportions of pigment and water may vary over wide limits depending on the method of application to 100 the fuel and the appearance desired in the product. In general, a ratio of one part of pigment to from one hundred to five hundred parts of water gives satisfactory results. If desired, the character of the suspension may be improved by subjecting the pigment to treatment in a colloid mill to increase the 105 degree of fineness and improve the dispersion

of the pigment in the water. The water employed in preparing the suspension may be pure water or it may be water from the mine in somewhat acid condition. The mine water 5 can be neutralized before the pigment is added thereto or the pigment may carry some acid neutralizing substance to correct the acidity of the water. After the suspension has been prepared it is brought into intimate 10 contact with the fuel in any desired manner, for example, by spraying or immersion. After the fuel has been thoroughly wet with the suspension it is drained to remove the excess thereof. The fuel may be permitted 15 to dry before shipment. Although the more or less complete removal of the water from the fuel probably enhances the permanency of the coating, we have determined that a satisfactory coating may be provided with- 20 out complete removal of the liquid before shipment or handling of the fuel. No special facilities for drying the fuel are required. The fuel treated as hereinbefore described has the coloring material or pigment distributed 25 over the surface area and it presents, therefore, a distinctive bluish appearance which differentiates it from fuel which has not been so treated. The coloring is sufficiently permanent to withstand ordinary handling and in- 30 cidental wetting of the fuel during transportation. Consequently the consumer can identify the fuel and can be certain, therefore, of the source and quality thereof.

Other pigments or colors may be similarly 35 employed. The fuel may be treated, for example, with aqueous suspensions of certain metal oxides, more particularly the oxides of heavy metals, such as zinc oxide, lead oxide, either in the form of litharge or red lead, and 40 iron oxide, either in its pure form or as one of the commercial pigments known as Venetian red, burnt sienna, or Indian red. Other available pigments are certain chromates of 45 heavy metals, such as chrome yellow, chrome orange or chrome green. These are merely examples and other oxides and other compounds of the metals may be utilized with similar advantage.

Another method of imparting the desired 50 appearance to the fuel consists in wetting it with a colloidal solution of iron hydroxide. For example ferric chloride crystals can be dissolved in the proportion of one-half of one 55 part to four parts by weight of crystals to one hundred parts of water. The resulting solution when boiled first forms a precipitate which afterwards disperses to a colloidal suspension. The fuel may be subjected to treatment with this suspension either by spraying 60 or immersion while the suspension is main- tained at a temperature preferably between 50° and 100° C. After the surplus liquid is drained off the fuel is coated with finely di- 65 vided iron oxide or hydroxide which adheres firmly to the surface and is not removed to

any extent during the subsequent handling of the fuel.

Another method of carrying out the invention consists in wetting the fuel with an aqueous suspension of a dye lake such as Carmine 70 40 or Tuscan Red. Tuscan Red can be produced by precipitating the natural dye hypernic on red iron oxide as a base. This pigment in finely divided form is then suspended in water in the ratio of one part of 75 pigment to from one hundred to five hundred parts of water. After a thorough treatment of the fuel with the aqueous suspension the surplus liquid is drained away and the fuel is left with a coating of the coloring material 80 which adheres firmly to the surface.

It is also possible to use insoluble dyes such as the so-called indanthrene colors. As an example a suspension of one part of Ponsol Red Violet 2BNX paste (du Pont) in one 85 hundred parts of water may be applied to the fuel by spraying or immersion. When the surplus liquid is drained from the fuel a coating of the dye will remain.

Another example of the method consists 90 in wetting the fuel with a suspension of a finely divided metal such as powdered aluminum, powdered copper or commercial bronze powder in a dilute aqueous solution of 95 a suitable binder. Sodium silicate may be used, for example, with some pigments. The ratio of powdered metal to the solution may be, for example, one part of the powder to from one hundred to five hundred parts of 100 solution, depending upon the effect to be produced. The fuel is treated by spraying or immersion with this suspension and the surplus solution is drained away, leaving the fuel coated with the metallic powder. The 105 permanency of the coating may be increased by treating the coated fuel with a very dilute solution of sulphuric acid or equivalent agent such as aluminum sulphate to harden the sodium silicate film.

Certain dyes which are insoluble in water 110 can be dissolved in oils such as gasoline, kero- sene, or other hydrocarbon oils, and utilized for the purpose of the present invention. For example, a 0.5% solution of the dye Oil 115 Blue Paste, of American Ahiline Products Company, or a 1% solution of the dye Oil Scarlet 6G, of National Aniline and Chemical Company, can be dissolved in gasoline or kerosene and applied to the fuel by spraying or by immersion as hereinbefore described. 120 When the surplus liquid is withdrawn and the solvent has evaporated the fuel is left with a superficial coating of a blue or red color which is not affected by water. A non- 125 volatile oil may be used in place of the vehicles mentioned, leaving a colored oily coating on the fuel. The fuel thus colored can be distinguished from ordinary fuel.

Similarly, solvents such as alcohol can be utilized with dyes soluble in alcohol but in- 130

soluble in water in about the same proportions. Thus, an alcohol solution of Oil Blue Paste or Oil Scarlet 6G can be applied to the fuel by spraying or immersion and the surplus liquid can be withdrawn. The alcohol evaporates readily, leaving the superficial color on the fuel which serves to distinguish it. Denatured alcohol can be used or ordinary 95% grain alcohol or absolute alcohol, although the cost of the latter solvents prohibits the use, thereof in ordinary commercial operations. Water-insoluble dyes which are soluble in acetone, benzol, toluol, etc., can be applied similarly to the fuel.

15 A class of dyes known as "basic" dyes may be applied to the fuel to provide a water-proof color by subjecting the dyes to the action of a mordant such as tannic acid. The color can be applied in either of two ways.

20 For example, the fuel is first wet with a solution of tannic acid and water, a 5% solution being suitable, and the fuel is then dried. It is wet with a water solution of a basic dye, for example, a 0.5% solution of Basic Blue 2B, and again dried. The dye is fixed by the tannic acid and is not affected by water. Other dyes of a similar character can be used likewise, for example, Basic Violet B, Crystal Violet, Safranine A, Phosphine and Rhodamine. These are merely examples of basic dyes which can be applied to the fuel for the purpose of the invention. The strength of the tannic acid solution and of the dye solution may be varied considerably without 30 affecting the results adversely.

Instead of the procedure as described the basic dye solution can be mixed with a solution of tannic acid. An insoluble finely divided precipitate or colloidal solution forms 40 which is a compound of the dye and the tannic acid or a lake. The precipitate or colloid remains in suspension and the suspension can be used by spraying or immersion to color the fuel. The precipitated lake acts as a pigment and is deposited on the surface of the fuel. After the fuel is dry the coloring material is not affected by water. As an example of this operation, a 5% aqueous solution of Basic Blue 2B is mixed with a 5% aqueous solution of tannic acid in the proportions of approximately 1:4. The resulting blue lake suspension is then applied to the fuel which is permitted to dry, leaving a bright blue color on the surface of the fuel. A red color can be imparted to the coal by mixing a 1% solution of Safranine A with a 5% solution of tannic acid in equal proportions. The red lake thus produced is applied to the fuel in the manner described and imparts a 50 superficial coating of red color thereto.

While commercially pure tannic acid is preferably employed, it is possible to use various extracts containing tannin, such as quebracho extract, chestnut extract, extract of 60 nut galls, etc., as mordants.

The basic dyes mentioned can be used similarly with soaps such as commercial rosin size (sodium resinate) or commercial soap. For example, the fuel is first immersed in a solution containing 5% of commercial rosin size by weight. Preferably, though not necessarily, the fuel is dried. It is then treated with a 0.5% solution of Basic Blue and is thereby given a water-proof coating of blue color. The fuel can be colored similarly in 75 a single operation by mixing a 1% water solution of Basic Blue 2B with a solution containing 5% of commercial rosin size by weight in equal proportions. The dye is precipitated as a finely divided compound which 80 can be maintained in suspension and applied thus to the fuel. When the fuel is dry a permanent water-proof colored coating is formed on the surface of the fuel.

Ordinary soap may be used in place of rosin size. For example, the fuel is first immersed in a solution containing 2% by weight of soap chips and dried. It is given a permanent color by immersing it in a 0.5% solution of Basic Blue. Alternatively, the dye solution 90 and the soap solution may be mixed and the resulting suspended color can be applied to the fuel by immersion or spraying. Pure salts of fatty acids such as sodium or potassium oleate, palmitate or stearate can be used 95 in place of ordinary soap or rosin size but the cost of these materials prohibits the use thereof in commercial operations.

The pigment or color may as hereinbefore indicated be applied to the fuel by blowing it thereon in a stream of air, the fuel being first moistened with water or with a solution containing, for example, sodium silicate. Conveniently the fuel may be caused to travel on a suitable conveyor past the air blast 100 which carries a pigment such as finely divided metal of the kind hereinbefore described. The moistened fuel is thus provided with a superficial coating of the pigment which is more or less permanently attached thereto 105 and serves to impart to the fuel a distinctive appearance.

As the surface of the coal is irregular and includes crests and valleys, the coloring material applied by the processes hereinbefore described will, in many cases, tend to settle in the valleys where it will remain in substantial amounts, and the crests or higher surfaces will be left substantially free from the coloring material, thereby causing the surface of the coal to be characteristically altered without causing it to lose its general appearance as such.

The numerous examples hereinbefore set forth are indicative of the wide range of possible variation in the character of the materials used and in the methods of application thereof to the fuel. In many instances the cost of the materials at present market prices would prevent the utilization thereof in the 130

commercial application of the invention. Nevertheless, in numerous instances the cost of coloring the fuel can be reduced to a point which permits the effective use thereof to accomplish the purpose of distinguishing fuel of high quality from the ordinary or poor grades of fuel which reach the market in large quantity.

It is unnecessary to coat all of the fuel. A quantity thereof may be coated in the manner and with any of the coloring materials hereinbefore described, and such coated fuel may be mixed in suitable proportions with other fuel to impart to the fuel the desired characteristic appearance. The proportions employed in mixing colored and uncolored fuel will depend upon the effect desired.

The invention affords a simple, satisfactory and economical procedure whereby fuel of any grade or from any source can be colored distinctively so that it can be recognized in the market as being of a certain grade or from a certain source. This ensures particularly that the consumer who purchases high grade

fuel will receive such product rather than inferior substitutes therefor. In avoiding substitution the producer as well as the consumer is benefitted because the producer can thus maintain the good-will based upon the production and sale of superior fuels.

We claim:

1. Coal having an irregular surface including crests and valleys, said coal having coloring material deposited in the valleys of the surface thereof in an amount sufficient to characteristically alter the appearance of the coal in bulk, but insufficient to cause the coal to lose its general appearance as coal.
2. Coal partly coated over its entire surface with coloring material, said coloring material being applied in an amount sufficient to characteristically alter the appearance of the coal in bulk but insufficient to cause the coal to lose its general appearance as coal.

In testimony whereof we affix our signatures.

GUSTAVUS J. ESSELEN, JR.  
MARK W. WEISS.